

Aug. 24, 1937.

H. M. CROWTHER

2,090,667

PROCESS OF AND APPARATUS FOR EXTRACTING SULPHUR FROM ORE

Filed Jan. 7, 1936



Fig. 1



Henry M. Crowther  
INVENTOR.

Fig. 2

## UNITED STATES PATENT OFFICE

2,090,667

## PROCESS OF AND APPARATUS FOR EXTRACTING SULPHUR FROM ORE

Henry M. Crowther, Los Angeles, Calif.

Application January 7, 1936, Serial No. 57,955

3 Claims. (Cl. 23—229)

Generally stated, the object of the invention is to provide an improved process and apparatus by which a given amount of sulphur ore, (usually 1000#) that has been previously crushed sufficiently so that the largest size pieces will pass the perforations of a one half inch mesh screen, is charged into an open-top cylindrical container which by the means provided is then lowered into and submerged in about five tons of molten sulphur contained in a tank having live steam heating drums also submerged in the sulphur bath to keep it at about 300 degrees Fahrenheit, and such immersing of the ore liquefies all of the elemental sulphur contained in the ore charge 10 within about 15 minutes, whereupon, by the means provided the ore container is raised above the level of the molten sulphur bath (but not above the rim of the submergence tank) and immediately the ore container is given one minute 15 of rotation at about 1000 R. P. M., which action centrifugally throws out fully 95% of the sulphur content of the ore, which liquefied sulphur during the rotary motion passes through the perforations of the double, spaced outer walls of the ore container, but in getting free is compelled to pass through a partition composed of metallic lead-wool which strains out all of the solid impurities and delivers commercially pure sulphur 20 into the supply of molten sulphur in the submergence tank, from which the excess outlets through an overflow conduit at any desired level. Means are provided whereby this system of treatment is accomplished without necessity of handling the hot ore containers, and also without loss of heat, as sulphur cools rapidly and cannot be given more than about 25 degrees of excess heat beyond its fusion point without injury to the quality of the product, which is the reason 25 for applying the centrifugal extraction cycle 30 immediately, and within the submergence tank without uncovering the tank for this purpose. The use of lead-wool is a special feature as it is not attacked by the sulphur and thus has an extra long life in the use employed. The invention does not consume any water (the live steam being used in return circuit) which is frequently 35 a great advantage where water is not plentiful.

The remarkably high recovery of the sulphur 40 accomplished by the invention renders the discharge of the tailings more convenient as customarily 10% or more of the sulphur is lost in the tailings by ordinary steam retorting methods depending on gravity flow of the sulphur from 45 the ore, and this excess loss of sulphur tends to

cement and cake the tailings in the treatment container.

I attain these objects by the mechanism illustrated in the accompanying drawing, in which:

Fig. 1 is a front elevation, in part sectionalized, 5 of a sulphur extracting apparatus embodying the principles of the invention.

Fig. 2 is a top view plan of the rotary ore container.

Similar numerals refer to similar parts 10 throughout the two views. As illustrated the invention comprises a circular metal tank 2, within which are positioned, and disposed near the walls of the tank a series of closed live-steam drums 3 which, in each case receive their hot steam supply 15 from a boiler source (not shown) by way of the connected pipes shown, each of which passes through the tank bottom to which each steam drum is anchored in leak proof manner. The tank is provided with an outlet pipe 4 which is 20 arranged as an overflow when tank is filled with molten sulphur to a certain fixed level, and this overflow pipe takes its load from the tank bottom but is prevented from acting as a siphon by the air vent 4A which, however may be capped and thus converting the overflow system into a siphon for purpose of draining the tank if desired at any time. Centrally anchored to the bottom of the tank on the outside is the guide 5, equipped with 25 a leak-proof packing gland, in which the solid rod 6 operates as a lift powered by the hydraulic cylinder 7 that receives its power from a source not illustrated; and this solid lift-rod has a fixed disc 8 anchored thereto positioned inside 30 of the tank bottom and serving as a rod movement limit. The ore charge for treatment is loaded into the open-top cylindrical container 10, and fixed centrally to the bottom, on the inside is the spindle seat 9 which journals on the spindle end of the hydraulic lift-rod and in this manner 35 the ore container is rotatably mounted and used in manner that will be more fully explained. The ore container has a perforated outer wall 11, and a similarly perforated, spaced inner wall 12, and between these two concentric spaced walls 40 is the spacer 13 which is removable, and sandwiched between the described spaced double walls is the partition or filling composed of metallic lead-wool serving as a molten sulphur filter. Oppositely positioned, in gravity dumping location 45 are fixed the dumping lugs 15, operable as explained later.

The tank is previously filled with a charge 50 of molten sulphur to the level of the dotted line 16, and kept molten by the steam heating drums 55

mentioned. The molten sulphur tank has a cover 17 centrally open to loosely fit the rotor plate 18 which serves as an automatic cover. The rotor plate is provided with a central drive shaft 19 journalled in the bearing block 20 which bearing block is fixed to the perpendicularly sliding frame 22, and with the rotor plate and its drive shaft held in place by the lock-collar 21. The sliding frame is carried by the timber uprights 23 and is counterbalanced by the dual counter-weight system 24 operable over the cable pulley means 25, illustrated.

The upper end of the rotor shaft 26 engages the rotor drive pulley 27 which is driven by a quarter turn belt from a friction clutch driving pulley, not shown; and the rotor drive pulley is retained against up and down movement by the cage 28 for the reason that in operation, during the introduction of the ore container into the sulphur bath tank, and its removal therefrom for dumping, the rotor drive shaft must slide longitudinally through the drive pulley, and to permit of this movement a long key-way 29 is formed in the drive shaft but the drive pulley 25 remains at all times slidingly keyed to the shaft by the fixed key 30 anchored in the pulley bore.

A pair of oppositely positioned dumping chairs 31 are provided to dump the tailings load of a treated charge by seating the dump pins of the container into a recess of the chairs, which operation will be more fully described.

In operating the process the tank is filled to its overflow level with pure molten sulphur and kept at proper temperature by applied steam heat, then the hydraulic lift rod is operated to raise the rotor plate five feet above the top of the tank and the rotor plate and its frame is locked at such point so as to give ample working room, then the ore container is ready for positioning on the spindle end of the hydraulic lift rod which is done by lowering the spindle and mounting the ore container thereon and lowering the container into the tank until its top is level with the top of the tank whereupon the container is loaded with ore from a dump car, and the container now loaded with a charge of ore is at once lowered by reversing the hydraulic lift until submerged in the molten sulphur bath, and immediately the rotor is lowered so that its plate closes the tank opening. After submergence of about 15 minutes the native sulphur of the ore charge will be completely liquefied, then the hydraulic lift is operated to raise the top rim of the ore container against the rotor which rotor assembly has about 100# of weight not counterbalanced and this provides ample friction to drive the container when the clutch of the rotor drive pulley is thrown in, whereupon the container, now above the level of the sulphur bath, is rotated at high speed for one minute and then the rotor drive clutch is released and as soon as the container movement ceases the hydraulic lift is operated to raise the ore container and the rotor assembly, at this time resting on the top rim of the container, to a height of six feet above the top rim of the sulphur bath tank at which point, out of the way, the rotor sliding carrier is locked, and the hydraulic lift is reversed to lower the container sufficiently to set its dumping axle pins in place in the seats of the dumping chairs, (fixed to the top of the tank, and arranged to swing into, and out of commission) whereupon the hydraulic lift again is lowered sufficiently to clear the container bottom 75 and leave the container free to swing on its

dumping trunnion system to a dumping position by reason of the overbalanced load in relation to its point of rotation, and thus the load of exhausted tailings is discharged into a dump-car, which, with its track is not illustrated, and after righting the container while still resting on the chairs the hydraulic hoist is raised to again seat the container on its spindle rod and the container is again lowered until its top rim is level with the tank top when it is again loaded with a fresh charge of ore from a dump-car and then again lowered to submerge the container and its load of ore in the molten sulphur bath in the tank, and the rotor assembly is allowed to lower by gravity to its position of rotation closing the tank opening, and ready to whirl the container after its bath, and repeat the cycle again and again continuously.

By providing some five tons of molten sulphur as a bath into which at fifteen minute intervals only one half a ton of cool ore is submerged the resulting lowering of the temperature of the bath is minimized within practical range, and with sufficient heat continuously supplied to the molten bath, ore may be treated in the manner described, continuously. It will be understood that in addition to using a bath of molten sulphur as a heat conducting agency for melting the sulphur of the ore being treated, the invention also uses the basic principle of passing through the ore simultaneously with the operation of removing the sulphur, a great excess of molten sulphur as a method of adding to the efficiency of the centrifugal whirling action practiced within the melting chamber or tank.

It is understood that usually a multiplicity of the units described will be employed, each unit treating about two tons of ore per hour if half ton loads are used.

Various changes may be made without departing from the spirit and scope of the invention.

I claim:

1. A process for extracting elemental sulphur from ore, comprising the placing of a load of sufficiently crushed ore in a container having perforated walls equipped with a filtering medium, and lowering the ore-loaded container to complete submergence in molten sulphur contained in a tank equipped with a removable cover and provided with facilities to maintain the molten sulphur at a temperature sufficient to melt the sulphur content of the ore charge, and leaving the ore submerged in the molten sulphur until all of the sulphur content of the ore has been melted, and thereafter raising the ore-container by means provided, free from the molten sulphur, and as soon as it is so raised rapidly rotating the container, by means provided, to cause the now molten sulphur of the ore, together with the excess sulphur of the submergence to be thrown centrifugally through the filter covered perforations of the ore-container to simultaneously filter the sulphur from the waste gangue or tailings and effect a high degree of extraction in the form of commercially pure sulphur.

2. In apparatus for extracting sulphur from ore, the combination of a tank equipped with removable cover, and suitable for containing molten sulphur at atmospheric pressure; means of heating and maintaining the sulphur in a properly molten condition; and provided with an overflow conduit automatically limiting level of the molten sulphur, and, also providing a discharge for excess accumulation of ore-recovered sulphur; and provided with a movable, filter-walled ore-con-

tainer equipped with lead-wool filtering medium, and having means provided for lowering the loaded ore-container into the molten sulphur, and means for raising the same, and, means for centrifugally spinning the loaded ore-container while in a raised position to recover, separate, and filter the sulphur content of the ore; and means provided for dumping the tailings, and reloading the ore-container with a fresh charge of ore ready

10 for treatment.

3. A non-pressure, dry process for extracting elemental sulphur from ore, which includes causing the sulphur content of the ore to be heat liquefied by submerging the ore in heat liquefied

sulphur which is maintained in a properly molten condition at atmospheric pressure, and without the addition of other reagents; and then removing the sulphur content of the ore thus rendered molten, together with any molten sulphur adhering to the charge from the submergence operation, while the molten sulphur being recovered is continually maintained, by heat provided and applied, in a heat liquefied condition, by means of centrifugal filtration employed at atmospheric pressure immediately upon removal of the ore from its treatment submergence by means provided.

HENRY M. CROWTHER.